

## UNITED STATES PATENT OFFICE.

CLIFFORD A. WOODBURY, OF MEDIA, PENNSYLVANIA, ASSIGNOR TO E. I. DU PONT DE NEMOURS & COMPANY, OF WILMINGTON, DELAWARE, A CORPORATION OF DELAWARE.

## AMMONIA DYNAMITE.

No Drawing.

Application filed April 13, 1922. Serial No. 552,067.

*To all whom it may concern:*

Be it known that I, CLIFFORD A. Woodbury, a citizen of the United States, and a resident of Media, in the county of Delaware and State of Pennsylvania, have invented a certain new and useful Ammonia Dynamite, of which the following is a specification.

My invention relates to an improvement in dynamites containing ammonium nitrate, and in particular to ammonia dynamites ranging in strength from about 45% to about 55%.

These grades of ammonia dynamite have in the past been manufactured on approximately the following formulas, and the resulting dynamites have had in general the properties listed below.

| Grade, about—                                                              | 45%  | 50%  | 55%  |
|----------------------------------------------------------------------------|------|------|------|
| Liquid explosive.....                                                      | 22   | 24   | 28   |
| Ammonium nitrate.....                                                      | 32   | 36   | 45   |
| Sodium nitrate and combustibles (e. g. wood pulp, starch, meal, etc.)..... | 46   | 40   | 27   |
| Density, 14" x 8" sticks per 50 lb. case.....                              | 102  | 102  | 102  |
| Velocity—in/sec.....                                                       | 3950 | 4200 | 4600 |
| Weight strength.....                                                       | 45   | 50   | 55   |
| Bulk strength.....                                                         | 44   | 49   | 54   |

In this tabulation and throughout this specification, the terms used have the following meanings:

The grade is based upon and is identical with the weight strength.

By weight strength is meant the explosive strength as determined by the ballistic mortar, expressed in terms of the nitroglycerine content of the straight nitroglycerine dynamite giving the same swing of the ballistic mortar.

The density is expressed in terms of the number of 14" x 8" sticks contained in 50 lbs. net weight of the finished dynamite, this being the method of stating density in the ordinary nomenclature of the explosives industry in this country.

By bulk strength is meant the strength per unit volume, or per stick, expressed in terms of the nitroglycerine content of the straight nitroglycerine dynamite having the same stick strength, straight nitroglycerine dynamite being assumed to have a density of 100 sticks, 14" x 8", per 50 lb. case.

The weight strength is considered therefore a criterion of the execution to be expected from a pound of the explosive, and

the bulk strength is a criterion of execution to be expected from a stick of the explosive.

By the term liquid explosive I mean to include nitroglycerine or nitrated glycol, or mixtures of these with nitrated sugars, nitrated polymerized glycerine, and nitrated aromatic compounds.

The dynamites described above have been a great improvement over previously used straight nitroglycerine dynamites of corresponding strengths from the standpoint of economy and safety, the ammonium nitrate being considerably cheaper than the nitroglycerine it replaces, and, in addition, by its presence, greatly reducing the inflammability of the powder and its sensitivity to shock.

For use in coal mines, ammonia dynamites having strengths within the range of 45% to 55% have also been made in which such materials as ammonium chloride or sodium chloride have been used for the purpose of reducing the temperature of explosion. This type of powder does not fall within the scope of my invention, however, on account of the excessive amounts of ammonium nitrate necessary in order to counterbalance the effect on strength produced by the use of flame temperature regulators.

By my invention I have produced substantial improvements over the previously used grades of dynamites in cost of manufacture and safety, and, in addition, in economy of use.

In my new dynamites I have gone farther than has heretofore been considered possible in the replacement of nitroglycerine with ammonium nitrate, for I have reduced the nitroglycerine content of these grades of powders to approximately 10%, which I have found to be the minimum required to properly sensitize the explosives.

The following table illustrates the composition of my new explosives and their approximate properties:

| Grade, about—                                            | 45%   | 50%   | 55%   | 100 |
|----------------------------------------------------------|-------|-------|-------|-----|
| Liquid explosive.....                                    | 9-12  | 9-12  | 9-12  |     |
| Ammonium nitrate.....                                    | 45-53 | 54-59 | 60-66 |     |
| NaNO <sub>3</sub> and combustible (wood pulp, etc.)..... | 38-43 | 33-34 | 25-28 |     |
| Density, about.....                                      | 117   | 121   | 125   |     |
| Velocity, about.....                                     | 3250  | 3300  | 3400  | 105 |
| Weight strength, about.....                              | 45    | 50    | 55    |     |
| Bulk strength, about.....                                | 34.5  | 36.0  | 38    |     |

A specific example of a 50% dynamite

made in accordance with my invention, would be a composition containing 10% of nitroglycerine, 56% of ammonium nitrate, and 34% of sodium nitrate and wood pulp or 5 other combustible material.

A comparison of these tabulated properties with those of the previously used dynamites will show a number of distinct advantages which the new dynamites possess, as 10 follows:—

1. The velocity of detonation is lower. This is an advantage where shattering power is undesirable.

2. The content of liquid explosive is decreased and that of ammonium nitrate is increased. Since liquid explosive will normally have a cost from two to four times that of ammonium nitrate depending on market conditions, there results a marked 20 saving in manufacturing cost per pound of finished explosive.

3. The increased number of sticks to the 50 lbs. of a lower cost dynamite constitutes a decided advantage to the user of the dynamite. Fifty pounds of my new explosive of 25 50% weight strength furnishes approximately 120 sticks of dynamite, each stick exhibiting a strength of approximately 36%. One stick of my new 50% dynamite should 30 do as much work as one stick of 35% ammonia dynamite as heretofore manufactured, but my new dynamite furnishes approximately 120 sticks as compared to 102 sticks of the 35% dynamite and, further- 35 more, the cost per stick is at least as low in the case of the former as it is for the latter under the conditions which have generally applied in this country.

In addition to these advantages, the further increase of ammonium nitrate content and decrease of liquid explosive content has further lowered the inflammability and sensitivity to shock of the finished explosive, thus contributing to safety in use.

Obviously, by means of minor changes in 45 the character of the ammonium nitrate or other ingredients, I may vary the density and velocity of my new explosive over a wide range without departing from the spirit of my invention.

50

I claim:

1. Blasting explosives ranging in strength from about 45% to 55% and containing from about 9% to 12% nitroglycerine, most 55 of the balance of the explosive strength being contributed by ammonium nitrate.

2. Blasting explosives ranging in strength from about 45% to about 55%, containing from about 9% to 12% of liquid explosive and from 45% to 65% of ammonium nitrate. 60

3. Blasting explosives ranging in strength from about 45% to about 55%, and containing from about 9 to 12% of liquid explosive and from about 45 to 65% of ammonium nitrate, the remainder comprising sodium nitrate and non-explosive combustible material. 65

4. Blasting explosives ranging in strength from about 45% to about 55%, containing from about 9% to 12% of liquid explosive 70 and from about 45% to 65% of ammonium nitrate, and having a density of 115 to 126, 14" x 8", cartridges per 50 lbs. of finished explosive.

5. A blasting explosive of 50% strength 75 containing from about 9% to 12% of a liquid explosive comprising nitroglycerine and from about 54% to 58% of ammonium nitrate.

6. A blasting explosive of 50% strength 80 containing from about 9% to 12% of a liquid explosive comprising nitroglycerine and from about 54% to 58% of ammonium nitrate, the remainder comprising sodium nitrate and non-explosive combustible material. 85

In testimony whereof I affix my signature.  
CLIFFORD A. WOODBURY.